

Nov. 3, 1942.

C. W. CUNO

2,300,488

ROOFING WITH SELF-CEMENTING BUTTS

Filed Jan. 17, 1941

2 Sheets-Sheet 1



INVENTOR.

Charles W. Cuno  
BY Mann, Brown & Co

ATTYS

Nov. 3, 1942.

C. W. CUNO

2,300,488

## ROOFING WITH SELF-CEMENTING BUTTS

Filed Jan. 17, 1941

2 Sheets-Sheet 2



BY Charles W. Curo  
Mann, Brown & Co.  
ATTYS.

## UNITED STATES PATENT OFFICE

2,300,488

## ROOFING WITH SELF-CEMENTING BUTTS

Charles W. Cuno, Wilmington, Ill., assignor to  
The Lehon Company, Chicago, Ill., a corpora-  
tion of Illinois

Application January 17, 1941, Serial No. 374,830

7 Claims. (CL 108—7)

A problem which has confronted the roofing industry for many years is the problem of keeping the lower ends of flexible shingles flat and tight against the roof. Only the upper parts of shingles are nailed and according to conventional practice the lower ends are left loose. The exposed portions cannot be nailed because this would cause leakage. Under some conditions these exposed loose shingle ends curl up. Occasionally a strong wind will catch under the loose ends of the shingles and blow the entire covering off of the roof.

A great deal of inventive thought has been devoted through the years to the effort of solving this problem. Of course, one expedient is to apply cement to the undersurface of the shingle as it is laid, but this greatly increases the cost of laying the shingles and hence is not ordinarily considered commercially practical unless in very windy areas where some securing means is considered necessary. Various schemes have been proposed for applying the cement to the shingles in manufacture but none of them have been satisfactory for the reason that there has been no practical way for keeping such cement from causing trouble by sticking in the bundle.

According to the present invention, the problem is solved in a manner which is thoroughly practical and at the same time is so exceedingly simple as to be thoroughly feasible from the manufacturing and cost standpoints. According to this invention, a cement is applied during manufacture which is of such nature that it will stick to other areas coated with the same cement but will not stick to areas not so coated. For convenience, this type of cement may be called a "cooperative adhesive." It needs cooperation between two cemented surfaces to adhere firmly. Each shingle is provided with a narrow band of the cooperative adhesive on its underside at the bottom thereof and another band on its face side. The position of the band at the top is such that it will not come in contact with the first mentioned band in the bundle and it will come in contact with and stick to the bottom of the overlying shingle in the overlapping position in which they are naturally laid.

Additional objects and advantages of the invention will be apparent from the following description and from the drawings, in which:

Fig. 1 is a face view of a roofing strip chosen for illustration of the present invention.

Fig. 2 is a back view of the same.

Fig. 3 is a view of a stack or bundle of the roofing strips with the upper strip curled back

10 to show the relationship between it and the strip therebelow.

Fig. 4 is a view showing the overlapped positions of the roofing elements on a roof with an upper element curved back to show the alignment of the adhesive on the back thereof with the adhesive on the front of the underlying strip.

Fig. 5 is an end elevation of a stack of the roofing elements shown in Figs. 1 to 4.

Fig. 6 is a sectional view taken approximately on the line 6—6 of a roof such as that shown in Fig. 4.

Fig. 7 is a diagrammatic representation of a suitable method and apparatus for forming the shingle strip of Figs. 1 to 4.

Figs. 8 and 9 are fragmentary detail views taken approximately on the lines 8—8 and 9—9 respectively, showing particularly the recessed rolls for receiving the adhesive bands.

20 A preferred form of the invention has been chosen for illustration and description, in compliance with section 4888 of the revised statutes, but persons skilled in the art will readily perceive other means for accomplishing the same results, and the claims are therefore to be construed as broadly as possible, consistent with the prior art.

As seen in Fig. 1, the shingle element chosen for illustration includes a head lap portion 11, at the lower end of which are formed a plurality of butt portions or tabs 12 separated by slots 13. Of course, the invention could be applied to other types of shingle or siding strips or to separate shingles. The roofing element illustrated is one conventional form of prepared roofing having a base of conventional roofing felt, conventionally saturated and coated with asphalt, and surfaced on its face with mineral granules and on its back with some adhesion-preventing medium, such as the conventional talc or mica flakes. It is preferred that this adhesion-preventing medium on the back comprise the thin creped tissue now being used for this purpose by The Lehon Company.

40 According to the present invention, a band 14 of cooperative cement (which will not adhere firmly except to like bands) is applied over the surfacing granules on the face of the shingle approximately at the bottom of the head lap 11. The band 14 extends the full length of the roofing strip. Another band 16 of the same cooperative cement is applied over the surfacing material on the back of the strip at the bottom thereof as seen in Fig. 2. The band 16 extends

the full length of the shingle strip except as it is interrupted by the slots 13.

As clearly seen from Figs. 3 and 5, the bands 14 and 16 do not come in contact with one another in the bundle and hence the shingles are not stuck together. The exposed face of the cooperative adhesive 14 comes in contact with the conventional non-adhesive surfacing or backing material on the strip above it and, as indicated by the expression "cooperative adhesive," it does not stick to this non-adhesive surface. Likewise, the band 16 of cooperative adhesive comes in contact only with the facing granules of the strip below it and does not adhere to these granules. Of course, in both instances the cement might cling slightly to the exposed surfaces as the shingles are pulled apart but not enough to render it difficult to separate the shingles or to disrupt either the cement or the surfacing material. As seen in Figs. 4 and 6, an entirely different action results from the overlapped displacement of the shingles in applying the shingles to a roof. In this instance the band 16 falls directly on the band 14 of the strip therebelow. The upper shingle strip should be pressed firmly against the lower shingle strip. When the two bands of cement 14 and 16 come in contact with one another in this manner and are pressed firmly together, they adhere together permanently and thus hold the butts or tabs 12 down tightly so that they will not curl or be blown up. This also tends to seal the roof so that wind cannot blow water upwardly under the tabs. It will be understood, of course, that the shingles are also secured in the conventional way by nails extending through the head lap portion and into the supporting roof structure.

The cooperative cement may comprise a wide variety of pressure-sensitive adhesive materials. It is probable that any of the pressure-sensitive adhesives could be used with a fair degree of satisfaction. It is preferred, however, that one be chosen which adheres a little less readily to other types of materials than some of the pressure-sensitive adhesives. The pressure-sensitive adhesives used on envelopes would be satisfactory, although they are relatively expensive.

One formula which would be satisfactory except for being more expensive than desired is the following:

|               | Parts    |
|---------------|----------|
| Milled rubber | 5 to 10  |
| Gasoline      | 75 to 80 |
| Mica          | 10       |

Other formulas of somewhat lower cost are the following, the first figures in formula (c) being at present preferred:

|                         | Parts          |
|-------------------------|----------------|
| (a) Milled rubber       | 10             |
| Tall oil pitch          | 50             |
| Benzol                  | 10             |
| Methyl abietate         | 5 to 10        |
| Talc                    | 10 to 15       |
| (b) Chlorinated rubber  | 5 to 10        |
| Hydrogenated rosin      | 25 to 35       |
| Hydrogenated gasoline   | 10 to 15       |
| Wax tailings            | 10 to 15       |
| Dihydro methyl abietate | 5 to 15        |
| Mica                    | 5 to 10        |
| (c) Rosin residue       | 45 or 40 to 60 |
| Rubber                  | 5 or 2 to 5    |
| Methyl abietate         | 15 or 10 to 20 |
| Hydrogenated gasoline   | 10 or 5 to 10  |
| Filler                  | 4 or 3 to 10   |

The filler in formula (c) is preferably powdered mica but mica, talc, clay and whiting are interchangeable as fillers in all of the formulas. Also, color may be added or substituted for other filler as desired. The rubber may be any scrap rubber, including chlorinated rubber, that is unvulcanized or only partly vulcanized. It is first dissolved in the hydrogenated gasoline (for which could be substituted gasoline, benzol or toluene), and the rosin residue is added next. Other resinous substances, such as those mentioned in the other formulas, could be used. The methyl abietate (known as "Abolyn") and the filler may be added subsequently. Any plasticizer which is a solvent for both the rubber and the rosin could be used instead, "Hercolyn" and dibutyl-phosphate being examples. The rosin residue is the residue from the steam distillation of rosin. One suitable form is that available from the Hercules Powder Company.

The cement is best applied immediately after the surfacing materials have been applied to the coated and saturated roofing felt. Thus, as seen in Fig. 7, the hot saturated and coated web 21 passes under a sprinkling trough 22 which supplies the facing granules and around a roll 23 which embeds these granules into the coating asphalt while at the same time a backing web 24 of creped tissue paper is applied from a roll 26. From the roll 23 the surfaced web 21 passes around rolls 27 and 28. As it does so, cement is printed onto the front and back surfaces of the web along the desired lines by rollers 29 which also run in contact with supply rollers 31 running with their lower portions below the cement level in cement reservoirs 32. Of course, conventional mica flakes or talc could be substituted for the paper but the adhesion would not be as good.

While the cement is wet, it will stick readily to non-adhesive materials such as the facing granules or the surfacing material on the back of the web or to the surfaces of the conveying rolls. However, it is conventional practice with roofing to carry the web through a cooler made up of a succession of rolls 36 which are usually water-cooled, and the cooling time thus provided will also serve to enable the cement to dry. It is of course necessary that the cement be kept out of contact with the surfaces of the rolls until it is dried enough so that it will not stick to them. To this end the rolls 36 are provided with annular grooves 38 positioned to receive the bands of freshly-applied cement 39. The cement bands will be quite thin and these grooves 38 may therefore be quite shallow.

It will be observed that according to the preferred process in Fig. 7 the cement is applied to the web while it is still quite hot, having just come from the coater before the granules are sprinkled thereon at 22. This is advantageous since it quickens the drying of the cement. To the same end the cement supply in the reservoirs 32 is preferably kept hot, say 150° F.

If desired, a shower of water may be applied from a shower pipe 41 across the face of the web as seen in Fig. 7. This speeds the cooling of the web and does not adversely affect the cement. In order to keep the water from running down the web into the cement reservoir 32, a pair of rolls 42 may be provided with the one closer to the reservoir higher than the other so that any excess water will run off adjacent the roll 42. As a matter of fact, since the temperature of the roofing is close to 300° F., a substantial amount of water will be quickly evaporated, and the

shower 41 can be so regulated that there will be little or no excess water to run off. The rolls 42 and 28 should of course be provided with grooves 38 such as those shown in Figs. 8 and 9 so that the cement will not stick to them. The rolls 27, 28 and 42 may all be rolls conventionally used in the manufacture of prepared roofing (except for the provision of the grooves 38 as mentioned), it having been common to provide a large roll at the position of the roll 27 and small shiftable rolls at approximately the positions of the rolls 28 and 42. The cementing rollers 29 may coat with these conventional rolls.

In Fig. 8 the band 39 on the underside of the shingle has been shown twice as wide as that on the upper side. This is because it is at the position in which the web is split longitudinally to form two shingle strips, each one including along one edge half of the cement band in question. It should be understood that the slots 13 are cut along the edges formed by this slitting so that this edge will be the bottom of the roofing strip in each instance. Of course, if preferred, two slightly separated narrow bands could be used in place of the one wide band and the slitting could be performed between them. This should be done if under any conditions it is found that there is trouble with sticking of the cement to the slitting wheel or to other parts when it is slit.

Although the invention has been illustrated in connection with square butt shingle strips cut longitudinally from the web, it will be apparent that the invention is also applicable to single shingles, hexagonal shingle strips, siding, rolls and all other analogous elements. In the case of some of these elements, it may be necessary to use a more complex cement painting roll to apply the cement in longitudinal registry with the ultimate cutting of the web. However, the simple cement-applying wheels can be used, at least on the back of the web, whenever the continuous cement bands will be staggered in the finished roofing element. This probably will include all elements having their horizontal dimensions cut longitudinally of the web. For example, in hexagon roofing, bands may be applied at the back of the web so positioned that one of them will be positioned adjacent each bottom edge. Although this will provide two bands on the back of each hexagon butt or tab, neither one of them will fall on the cement band on the underlying head lap portion in the bundle. In this event the head lap portions or the portions lying under the tabs in the finished roof may be provided with two bands, one coinciding with each band on the back of the butt. It is only these bands on the head lap portion that need to be registered in order to keep them from being visible between the tabs of the overlying shingle. It will be observed from Fig. 4 that the band 14 is visible between the tabs 12 of the overlying shingle, but the area of visibility is so small that this will not be noticeable.

From the foregoing it is seen that the problem of adequately and permanently securing the exposed butts of roofing elements to the roof in an inexpensive manner which will not make more expensive the application of the elements to the roof has been solved. The cooperative cement may be applied in narrow zones and with simple apparatus so that it will not be very costly. It is of such nature that it will not cause any firm adhesions in the bundle where the bands do not come in contact with one another and yet it

will secure the butts firmly and permanently when the bands of cooperative adhesive are pressed together on the roof.

I claim:

- 5 1. A roofing element having on its surfaces areas of cement characterized by the ability to stick to other cemented areas but not to areas free of the cement, one of said areas being on the front of the element and one being at a position on the back of the element near its bottom edge staggered so as not to contact the cemented area on the front of an adjacent element in a bundle but so as to come in contact with the cemented area on the front of an underlying element in the proper method of laying elements on a roof.
- 10 2. A roofing element having on its surfaces areas of cement characterized by the ability to stick to other cemented areas but not to areas free of the cement, one of said areas being on the front of the element and one being at a position on the back of the element staggered so as not to contact the cemented area on the front of an adjacent element in a bundle but so as to come in contact with the cemented area on the front of an underlying element in the proper method of laying elements on a roof.
- 15 3. A roofing element having on its surfaces areas of cement characterized by the ability to stick to other cemented areas but not to areas free of the cement, one of said areas being on the front of the element and one being at a position on the back of the element near its bottom edge staggered so as not to contact the cemented area on the front of an adjacent element in a bundle but so as to come in contact with the cemented area on the front of an underlying element in the proper method of laying elements on a roof, said areas being in the form of substantially continuous parallel bands.
- 20 4. A roofing element having on its surfaces areas of cement characterized by the ability to stick to other cemented areas but not to areas free of the cement, one of said areas being on the front of the element and one being at a position on the back of the element near its bottom edge staggered so as not to contact the cemented area on the front of an adjacent element in a bundle but so as to come in contact with the cemented area on the front of an underlying element in the proper method of laying elements on a roof, said areas being so staggered as to come in contact with one another in a bundle only if like faces are put together with top edges together and bottom edges together.
- 25 5. A roofing element having first and second faces, an adhesive area on the first face, and a cooperative area on the second face, the disposition of these two areas being such that, in proper laying of a plurality of such roofing elements on a roof in overlapping relationship, the adhesive area of one will come in contact with the cooperative area of the other but when properly arranged in a bundle these areas will not come in contact with one another, the areas which will come in contact with each of said first-named areas in a bundle being of such nature as not to adhere to the contacting area.
- 30 6. A roofing element having first and second faces, an adhesive area on the first face, and a cooperative area on the second face, the disposition of these two areas being such that, in proper laying of a plurality of such roofing elements on a roof in overlapping relationship, the adhesive area of one will come in contact with the cooperative area of the other adjacent the bottom

edge of the upper element but when properly arranged in a bundle these areas will not come in contact with one another, the areas which will come in contact with each of said first-named areas in a bundle being of such nature as not to adhere to the contacting area.

7. A roofing element having first and second faces, an adhesive area on the first face, and a cooperative area on the second face, the disposition of these two areas being such that, in proper laying of a plurality of such roofing elements on a roof in overlapping relationship, the adhesive

area of one will come in contact with the cooperative area of the other but when properly arranged in a bundle these areas will not come in contact with one another, the areas which will come in contact with each of said first-named areas in a bundle being of such nature as not to adhere to the contacting area, the adhesive and cooperative areas being so staggered as to come in contact with one another in a bundle only if like faces are put together with top edges together and bottom edges together.

CHARLES W. CUNO.